# EUROPEAN PATENT SPECIFICATION

(11) **EP 2 601 321 B1**
(45) Date of publication and mention of the grant of the patent: **29.11.2017**
(21) Application number: 11760871.1
(22) Date of filing: 04.08.2011
(51) Int. Cl.: C21D 7/06, C23C 8/80, C21D 1/06, C23C 8/22, C21D 11/00

(54) **A METHOD FOR SHOT PEENING A GAS CARBURISED STEEL**
KUGELSTRAHLVERFAHREN FÜR EINEN UNTER GAS AUFGEKOHLTEN STAHL
PROCÉDÉ DE GRENAILLAGE D'UN ACIER CÉMENTÉ AU GAZ

(30) Priority: 05.08.2010 JP 2010176681
(43) Date of publication of application: 12.06.2013
(73) Proprietor: Sintokogio, Ltd., Nagoya-shi, Aichi 450-0002 (JP)
(72) Inventor: KOBAYASHI, Yuji, Toyokawa-shi Aichi 442-8505 (JP); TSUJI, Toshiya, Toyokawa-shi Aichi 442-8505 (JP)
(74) Representative: Thum, Bernhard
(86) International application number: PCT/JP2011/004416
(87) International publication number: WO 2012/017658

(56) References cited:
- JP-A- 5 140 726
- US-B1- 6 655 026
- OGAWA K ET AL: "Theoretical prediction of residual stress induced by shot peening and experimental verification for carburized steel", ZAIRYO/JOURNAL OF THE SOCIETY OF MATERIALS SCIENCE, JAPAN DECEMBER 1999 SOC MATER SCI, JAPAN, vol. 48, no. 12, December 1999 (1999-12), pages 1360-1366, XP002665725,

## Description

### Technical Field

The present invention relates to a method for shot peening. Specifically, it relates to a method for shot-peening a gas carburized steel.

### Background Art

Conventionally, shot peening has been known to produce compressive residual stresses and to increase hardness to improve the fatigue strength of gears (see authored by the Society of Shot Peening Technology of Japan; Fatigue of Metals and Shot Peening; published by Gendai Kogaku-sha; 2004). Further, to achieve high fatigue strength aimed at reducing the weight of parts, a method for increasing compressive residual stresses produced by shot peening has been known (see Kazuyoshi Ogawa and Takashi Asano; Theoretical Prediction of Residual Stress Produced by Shot Peening for Hardened Steel; Transactions of JSSR, No. 48 (2003) pp. 31-38).

However, in these studies only the mean values of the hardness on the surface of, or near the surface of, the material are focused on. Thus the methods by these studies are difficult to be applied to a gas carburized steel that has a soft layer on the surface, since residual stresses are affected by plastic deformations caused by the collision of shot media and the mechanical properties of the processed steels that relate to the suppression of the plastic deformation. In the article "Theoretical Prediction of Residual Stress Induced by Shot Peening and Experimental Verification for Carburized Steel", by Kazuyoshi Ogawa and Takashi Asano, a model has been developed to predict the maximum and peak depth of compressive residual stress in carburized steel due to shot peening.

### Disclosure of the Invention

The object of the present invention is to provide a method for shot peening for producing high compressive residual stresses in a gas carburized steel that has a soft layer on the surface. In this method, a depth where the maximum compressive residual stress is generated is estimated, and no data on the hardness on the surface or near the surface is used.

The method for shot peening of the first aspect of the present invention is to produce a compressive residual stress in a processed steel by peening shot media onto the processed steel. The processed steel comprises a gas carburized steel having a hardness of 750HV or higher at the depth z, where the maximum compressive residual stress is generated. The depth z is estimated by using Equations (1) to (4) below. The shot media have a hardness that is above that of the processed steel by 50HV or more. $α = \frac{1}{2 {E *}^{\frac{1}{5}}} {\left(\frac{5 π}{4}\right)}^{\frac{1}{5}} D {ρ}^{\frac{1}{5}} {V}^{\frac{2}{5}}$ $\frac{1}{E *} = \frac{1 - {{v}_{1}}^{2}}{{E}_{1}} + \frac{1 - {{v}_{2}}^{2}}{{E}_{2}}$ $z = 0.48 Kα$ $K = 1.25$ where
α: contact radius by shot media (m),
p: specific gravity of shot media (kg/m³),
D: diameter of shot media (m),
v: shot speed (m/s),
E*: equivalent elastic modulus
E₁: Young's modulus of the processed steel (Pa),
v₁: Poisson's ratio of the processed steel,
E₂: Young's modulus of shot media (Pa),
v₂: Poisson's ratio of shot media,
K: constant, and
z: depth where the maximum compressive stress is generated (m).

The method for the shot peening of the second aspect of the present invention is characterized in that the diameters of shot media are in the range from 0.2 mm to 1.0 mm in the method for the shot peening of the first aspect.

By the method for the shot peening of the first aspect of the present invention, the position where the maximum compressive residual stress is generated is estimated by multiplying the depth by a constant. The depth is determined as the depth where the maximum stress is generated by the collision of shot media. By shot-peening a gas carburized steel a maximum compressive residual stress that is equal to, or more than, 1,600 MPa, is produced. At that depth the gas carburized steel has a hardness that is equal to, or more than, 750HV. The shot media have a hardness that is above that of the processed steel by 50HV or more. Thus the processed steel is processed to have a high fatigue strength. That is, by estimating the depth z, where the maximum compressive stress is generated, from Equations (1) to (4), it is possible to produce a high compressive residual stress in a gas carburized steel that has a soft layer.

By the method for the shot peening of the second aspect of the present invention, since the diameters of shot media are in the range from 0.2 to 1.0 mm, the maximum compressive residual stress can be securely produced in the processed steel

The present invention will become more fully understood from the detailed description given below. However, the detailed description and the specific embodiment are illustrations of desired embodiments of the present invention, and are described only for an explanation. Various possible changes and modifications will be apparent to those of ordinary skill in the art on the basis of the detailed description.

### Brief Description of Drawings

Fig. 1 is a graph showing the distribution of the hardness of the processed steels that were used in the embodiments of the present invention.
Fig. 2 is a table showing the conditions and the results of the shot peening that were used in the embodiments of the present invention.
Fig. 3 is a graph showing the relationship between the estimated values and measured values where the maximum compressive residual stress is generated.
Fig. 4 is a graph showing the relationship between the differences between the hardness of shot media from the hardness at the depth where the maximum residual stresses is generated and the maximum compressive residual stresses.

### Best Mode for Carrying out the Invention

Below, the embodiments of the present invention are described with reference to the drawings.

Fig. 1 is a graph showing the distribution of the hardness of the processed steels that were used in the embodiments. The abscissa denotes depths (micrometer) from the surface of the steel, and the ordinate denotes the Vickers hardness. A gas carburized steel is used for the processed steels. In the drawing, "TP. A" and "TP. B" denote the steels which have been tempered at 180 degree C and 180 degree C, respectively.

Fig. 2 is a table showing the conditions and the results of shot peening that were used in the embodiments. A compressive-air shot peening system was used. Shot media that have a hardness of 700HV to 1,000HV and diameters (the mean diameters) of 0.2 to 1.0 mm were used.

The
"Maximum σ _{R}¹¹
in the table denotes the maximum compressive residual stresses in the processed steels. The compressive residual stresses were measured by using a micro-stress analyzer that is available from Rigaku Corporation
(X-ray tube: Cr-Kα; diffractive surface: (220); stress constant: -318MPa/deg; Bragg angle of the strain-free 2θ: 156.4 °).

The "Depth of Peak" in the table denotes the depth from the surface where the maximum compressive residual stress is generated. The "Hardness at Peak" denotes the hardness at the "Depth of Peak," i.e., the Vickers hardness of the processed steels at the depth where the maximum compressive residual stress is generated. The "Relative Hardness" denotes the differences between the hardness of shot media and that of the processed steels, specifically the value that is calculated by subtracting the hardness at peak of the processed steels from the hardness of shot media. As shown in the table, if the relative hardness is 50HV or more, the maximum compressive residual stress of - 1,600 MPa or more can be obtained. The maximum compressive residual stress of - 1,600 MPa is a typical value that is required for gear materials.

Fig. 3 is a graph showing the estimated values and measured values of the depths where the maximum compressive residual stress is generated. The estimated values are calculated by using the following Equations (1) to (4). $α = \frac{1}{2 {E *}^{\frac{1}{5}}} {\left(\frac{5 π}{4}\right)}^{\frac{1}{5}} D {ρ}^{\frac{1}{5}} {V}^{\frac{2}{5}}$ $\frac{1}{E *} = \frac{1 - {{v}_{1}}^{2}}{{E}_{1}} + \frac{1 - {{v}_{2}}^{2}}{{E}_{2}}$ $z = 0.48 Kα$ $K = 1.25$
α: contact radius by shot media (m),
ρ: specific gravity of shot media (kg/m³),
D: diameter of shot media (m),
v: shot speed (m/s),
E*: equivalent elastic modulus
E₁: Young's modulus of the processed steel (Pa),
v₁: Poisson's ratio of the processed steel,
E₂: Young's modulus of shot media (Pa),
v₂: Poisson's ratio of shot media,
K: constant, and
z: depth where the maximum compressive stress is generated (m).

As shown in Fig. 3, the estimated values where the maximum compressive residual stress is generated are generally coincident with the measured values. That means that the depths where the maximum compressive residual stress is generated can be estimated by multiplying the depth where the maximum stress is generated under contact stresses caused by the collision of shot media, by the constant K.

Fig. 4 is a graph showing the relationship between the differences between the hardness of shot media and the hardness at the depth where the maximum compressive residual stress is generated. Specifically, it shows the values (the relative hardness) that are calculated by subtracting the hardness of the processed steels at the peak depth from the hardness of shot media on the abscissa and the maximum compressive residual stresses (MPa) of the processed steels on the ordinate.

As shown in Fig. 4, if the value that is calculated by subtracting the hardness of the processed steels at the peak depth from the hardness of shot media is less than 50HV, the maximum compressive residual stress does not re ach -1,600 MPa. This is because shot media are subject to plastic deformation when they are shot onto the processed steel. Thus energy is insufficiently transmitted from shot media to the processed steel.

On the contrary, if the value that is calculated by subtracting the hardness of the processed steels at the peak depth from the hardness of shot media is 50HV or more, the maximum compressive residual stress exceeds -1,600 MPa. Since the maximum compressive residual stress is generally expressed as a minus value, that means that the absolute value exceeds 1,600 MPa. This is because shot media are seldom subject to plastic deformation when they are shot onto the processed steel. Thus sufficient energy is transmitted from shot media to the processed steel.

Further, as shown in Fig. 4, if the hardness of the processed steel at the depth where the maximum compressive residual stress is generated is less than 750HV, the maximum compressive residual stress does not reach -1,600 MPa even when the value that is calculated by subtracting the hardness of the processed steels at the peak depth from the hardness of shot media is 50HV or more. The maximum compressive residual stress to be produced in a steel is known as being limited by the yield strength of the steel. The yield strength is proportional to the hardness. Thus, unless the hardness of the processed steel at the depth where the maximum compressive residual stress is generated is 750HV or more, the yield strength that is required to produce the maximum compressive residual strength of -1,600 MPa cannot be ensured.

The threshold for the difference in the hardness of shot media and the processed steels, i.e., 50HV, is determined as follows. As shown in Fig. 4, the maximum compressive residual stresses are shown in relation to the values that are calculated by subtracting the hardness of the processed steels at the "Depth of Peak" from the hardness of shot media. An estimated curve is drawn by the least square method. Based on the curve the threshold is determined. The threshold for the hardness at the depth where the maximum compressive residual stress is generated, i.e., 750HV, is determined as follows. The maximum compressive residual stresses are shown in relation to the hardness of the processed steels. An estimated curve is drawn by the least square method. Based on the curve the threshold is determined.

As discussed above, in the embodiments of the present invention processed steels are used that have a hardness that is greater than 750HV at the depth z, where the maximum compressive residual stress is generated. The depth z is estimated from Equations (1) to (4). The shot media that have the hardness that is greater than that of the processed steels at the depth z by 50HV or more are shot onto the processed steels. In these ways a compressive residual stress is produced in the processed steels. In other words, the depth where the maximum compressive residual stress is generated is estimated by multiplying the depth where the maximum stress is generated under contact stresses caused by the collision of shot media by the constant K. The processed steels that have a hardness at that depth that exceeds 750HV are used. The shot media that have a hardness that is greater than that of the processed steels at the estimated depth by 50HV or more are shot onto the processed steels. As a result, a maximum compressive residual stress that is 1,600 MPa or more can be produced in the processed steels. Thus the processed steels can be improved in fatigue strength. That is, by estimating the depth z, where the maximum compressive residual stress is generated, from Equations (1) to (4), a high compressive residual stress can be produced in a gas carburized steel that has a soft layer.

Further, by having the diameters of shot media being in the range from 0.2 mm to 1.0 mm, a maximum compressive residual stress that is 1,600 MPa or more can be securely produced in the processed steels.

In this invention, any shot media can be used. However, shot media made of steels, etc., are preferable.

## Claims

1. A method for shot peening,
wherein a processed steel comprises a gas carburized steel that has hardness at 750HV or more at a depth z, where a maximum compressive residual stress is generated, the depth z being estimated by using Equations (1) to (4), and
wherein shot media that have a hardness that is greater than the hardness of the processed steel by 50HV or more are shot onto the processed steel to produce a compressive residual stress in the processed steel: $α = \frac{1}{2 {E *}^{\frac{1}{5}}} {\left(\frac{5 π}{4}\right)}^{\frac{1}{5}} D {ρ}^{\frac{1}{5}} {V}^{\frac{2}{5}}$ $\frac{1}{E *} = \frac{1 - {{v}_{1}}^{2}}{{E}_{1}} + \frac{1 - {{v}_{2}}^{2}}{{E}_{2}}$ $z = 0.48 Kα$ $K = 1.25$ where
α: contact radius by shot media (m),
ρ: specific gravity of shot media (kg/m³),
D: diameter of shot media (m),
V: shot speed (m/s),
E*: equivalent elastic modulus
E₁: Young's modulus of the processed steel (Pa),
v₁: Poisson's ratio of the processed steel,
E₂: Young's modulus of shot media (Pa),
v₂: Poisson's ratio of shot media,
K: constant, and
z: depth where the maximum compressive stress is generated (m).

2. The method for shot peening of claim 1, wherein diameters of the shot media are in a range from 0.2 mm to 1.0 mm.

## Patentansprüche

1. Kugelstrahlverfahren,
bei dem ein bearbeiteter Stahl einen in Gasatmosphäre aufgekohlten Stahl mit einer Härte von 750 HV oder darüber in einer Tiefe z umfasst, wobei eine maximale Druckeigenspannung erzeugt wird und die Tiefe z anhand der Gleichungen (1) bis (4) ermittelt wird, und
wobei Strahlmedien mit einer Härte, die um 50 HV oder mehr höher ist als die Härte des bearbeiteten Stahls auf den bearbeiteten Stahl geschleudert werden, um eine Druckeigenspannung im bearbeiteten Stahl zu erzeugen: $α = \frac{1}{2 {E *}^{\frac{1}{5}}} {\left(\frac{5 π}{4}\right)}^{\frac{1}{5}} D {ρ}^{\frac{1}{5}} {V}^{\frac{2}{5}}$ $\frac{1}{E *} = \frac{1 - {{v}_{1}}^{2}}{{E}_{1}} + \frac{1 - {{v}_{2}}^{2}}{{E}_{2}}$ $z = 0.48 Kα$ $K = 1.25$ wobei:
α: Kontaktradius durch Strahlmedien (m);
p: spezifisches Gewicht der Strahlmedien (kg/m³);
D: Durchmesser der Strahlmedien (m);
V: Geschwindigkeit der Strahlmedien (m/sec);
E*: äquivalenter Elastizitätsmodul;
E₁: Young'scher Modul des bearbeiteten Stahls (Pa);
v₁: Poisson-Verhältnis des bearbeiteten Stahls;
E₂: Young'scher Modul der Strahlmedien (Pa);
v₂: Poisson-Verhältnis der Strahlmedien;
K: Konstante; und
z: Tiefe, in der die maximale Druckeigenspannung erzeugt wird (m).

2. Kugelstrahlverfahren nach Anspruch 1, wobei die Durchmesser der Strahlmedien im Bereich von 0,2 mm bis 1,0 mm liegen.

## Revendications

1. Procédé de grenaillage,
dans lequel un acier traité comprend un acier carburé au gaz qui a une dureté à 750 HV ou plus à une profondeur z, où une contrainte de compression résiduelle maximum est générée, la profondeur z étant estimée en utilisant les Équations (1) à (4), et
dans lequel une grenaille qui a une dureté qui est supérieure à la dureté de l'acier traité de 50 HV ou plus est projetée sur l'acier traité pour produire une contrainte de compression résiduelle dans l'acier traité : $α = \frac{1}{2 {E *}^{\frac{1}{5}}} {\left(\frac{5 π}{4}\right)}^{\frac{1}{5}} D {ρ}^{\frac{1}{5}} {V}^{\frac{2}{5}}$ $\frac{1}{E *} = \frac{1 - {v}_{1}^{2}}{{E}_{1}} + \frac{1 - {v}_{2}^{2}}{{E}_{2}}$ $z = 0 , 48 Kα$ $K = 1 , 25$ où
α : rayon de contact par la grenaille (m),
ρ : poids spécifique de la grenaille (kg/m³),
D : diamètre de la grenaille (m),
V : vitesse de grenaillage (m/s),
E* : module d'élasticité équivalent,
E₁: module de Young de l'acier traité (Pa),
v₁ : coefficient de Poisson de l'acier traité,
E₂ : module de Young de la grenaille (Pa),
v₂ : coefficient de Poisson de la grenaille,
K : constante, et
z : profondeur où la contrainte de compression maximum est générée (m).

2. Procédé de grenaillage selon la revendication 1, dans lequel des diamètres de la grenaille sont dans une plage de 0,2 mm à 1,0 mm.
